

1

3,525,622

**LIGHT-SENSITIVE SILVER HALIDE EMULSIONS**  
Jozef Frans Willems, Wilrijk-Antwerp, and Albert Lucien Poot, Kontich, Belgium, assignors to Gevaert-Agfa N.V., Mortsel, Belgium, a Belgian company  
No Drawing. Filed Mar. 15, 1967, Ser. No. 623,207  
Claims priority, application Great Britain, Mar. 15, 1966,

11,345/66

Int. Cl. G03c 1/08, 1/34

U.S. Cl. 96—102

5 Claims

### ABSTRACT OF THE DISCLOSURE

Silver halide emulsion layers in photographic material are stabilized against spontaneous fogging during storage and/or development by the inclusion therein of a compound having the following general formula:



This invention relates to light-sensitive silver halide emulsions.

Light-sensitive silver halide emulsions are in general characterized by their sensitivity, gradation and fog.

As is well-known, sensitivity, gradation and fog can be regulated by the way of preparing the silver halide and the use of special chemical ingredients effecting a desired improvement or result. Addenda to the emulsion which are of particular importance for the stability of the light-sensitive characteristics of a silver halide emulsion are the so-called "stabilizers."

Stabilizers or antifoggants protect the light-sensitive silver halide emulsions against spontaneous growth of fog during prolonged storage or storage at high temperatures and humidities or during development to maximum contrast and speed.

According to the present invention, photographic silver halide emulsions can be stabilized against the formation of spontaneous fog by incorporating in the emulsions certain silver complexing agents, more particularly heterocyclic hydrazone compounds which can be represented by the following general formula (I):



(I)

wherein:

R represents a hydrogen atom or an alkyl radical,  
Z represents the atoms necessary for completing a heterocyclic ring. Said ring may contain in addition to the nitrogen atom one or more hetero atoms e.g. oxygen, nitrogen, selenium, or sulphur atoms forming a known heterocyclic ring such as those of the thiazole series (e.g. thiazole, 4-methylthiazole, 4-methyl-5-carbethoxythiazole, 4-phenylthiazole, 5-methylthiazole, 5-phenylthiazole, 4-(p-tolyl)thiazole, 4-(p-bromophenyl)thiazole, 4,5-dimethylthiazole, 4,5-diphenylthiazole, 4-(2-thienyl)thiazole, 4-(m-nitrophenyl)thiazole, those of the benzothiazole series (e.g. benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 6-sulfonic acid benzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole,

2

4,5,6,7-tetrahydrobenzothiazole, 5,6-dimethoxybenzothiazole, 5,6-dioxymethylenebenzothiazole, 5-hydroxybenzothiazole, 6-hydroxybenzothiazole, 5,6-dimethylbenzothiazole), those of the naphthothiazole series (e.g. naphtho[2,1-d]thiazole, naphtho[1,2-d]thiazole, 5-methoxynaphtho[1,2-d]thiazole, 5-ethoxynaphtho[1,2-d]thiazole, 8-methoxynaphtho[2,1-d]thiazole, 7-methoxynaphtho[2,1-d]thiazole), those of the thionaphtho[7,6-d]thiazole series (e.g. 7-methoxythionaphtho[7,6-d]thiazole), those of the thiadiazole series (e.g. 4-phenylthiadiazole, 4-ethylthiadiazole, 4-benzylthiadiazole, 4-benzylsulphonylthiadiazole), those of the oxazole series (e.g. 4-methyloxazole, 5-methyloxazole, 4-phenyloxazole, 4,5-diphenyloxazole, 4-ethyloxazole, 4,5-dimethyloxazole, 5-phenyloxazole), those of the benzoxazole series (e.g. benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 6-methoxybenzoxazole, 5-hydroxybenzoxazole, 6-hydroxybenzoxazole), those of the naphthoxazole series (e.g. naphtho[2,1-d]oxazole, naphtho[1,2-d]oxazole), those of the selenazole series (e.g. 4-methylselenazole, 4-phenylselenazole), those of the benzoselenazole series (e.g. benzoselenazole, 5-chlorobenzoselenazole, 5-methoxybenzoselenazole, 5-hydroxybenzoselenazole, 4,5,6,7-tetrahydrobenzoselenazole), those of the naphthoselenazole series (e.g. naphtho[2,1-d]selenazole, naphtho[1,2-d]selenazole), those of the 2-quinoline series (e.g. the quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline, etc.), those of the pyrimidine series, those of the quinoxaline series, those of the quinazoline series, those of the 1-phthalazine series, those of the 2-pyridine series (e.g. pyridine, 5-methylpyridine, 5-nitropyridine), those of the benzimidazole series (e.g. 1-ethylbenzimidazole, 1-phenylbenzimidazole, 1-ethyl-5,6-dichlorobenzimidazole, 1-hydroxy-ethyl-5,6-dichlorobenzimidazole, 1-ethyl-5-chlorobenzimidazole, 1-ethyl-5,6-dibromobenzimidazole, 1-ethyl-5-chloro-6-amino-benzimidazole, 1-ethyl-5-chloro-6-bromobenzimidazole, 1-ethyl-5-phenylbenzimidazole, 1-ethyl-5-fluorobenzimidazole, 1-ethyl-5,6-difluorobenzimidazole, 1-ethyl-5-cyanobenzimidazole, 1-( $\beta$ -acetoxyethyl)-5-cyanobenzimidazole, 1-ethyl-5-fluoro-6-cyanobenzimidazole, 1-ethyl-5-acetylbenzimidazole, 1-ethyl-5-chloro-6-fluorobenzimidazole, 1-ethyl-5-carboxybenzimidazole, 1-ethyl-7-carboxybenzimidazole, 1-ethyl-5-carbethoxybenzimidazole, 1-ethyl-5-sulphamyl-benzimidazole, or 1-ethyl-5-N-ethylsulphamylbenzimidazole, and

Z' represents the necessary atoms to close a heterocyclic ring containing as heteroatoms one or more nitrogen atoms e.g. a 2H-pyrrole, imidazole, benzimidazole, 1-H-indazole, pyrazole, triazole, pyridine, pyrazine, pyrimidine, s-triazine, isoquinoline, quinoline, phthalazine, quinoxaline, quinazoline, cinnoline, phenanthridine or condensed ring systems containing said nuclei e.g.  $\beta$ -purine, pteridine,  $\beta$ -carboline and phenanthroline.

Compounds according to Formula I above can be prepared according to one of the methods described in our

Belgian patent specification 679,558 filed Apr. 15, 1966.

Of the compounds set forth in the following Table 1, those compounds designated 1 and 2 can be prepared in the manner described by Geldard and Lions, J. Am. Chem. Soc. 84, 2262-3 (1962), while compound number 46 can be prepared in the manner described by Lions and Martin, J. Am. Chem. Soc. 80, 3858-65 (1958). The other hydrazone compounds comprehended by general Formula I above can be prepared by the condensation of a hydrazino derivative which corresponds to the heterocyclic ring structure Z, i.e. that ring structure to the right-hand of Formula I carrying a hydrazino group with an aldehyde derivative corresponding to the heterocyclic ring structure Z', i.e. that ring structure at the left-hand of Formula I carrying an aldehyde group. The general method of carrying out such condensation is as follows. 0.025 mole of hydrazino derivative dissolved or suspended in 25 ccs. of ethanol are mixed with 0.025 mole of aldehyde derivative dissolved in 25 ccs. of ethanol. The reaction mixture is refluxed on a boiling water bath for 30 min. After cooling, the formed precipitate is sucked off and washed with ethanol and dried. In most cases the obtained product is pure enough so that no further purification is necessary. Only the compound 15 is recrystallized from ethylene glycol monomethyl ether.

In the following Table 1 compounds which are particularly suited for use according to the present invention are listed.





40. Some of the antifoggants described above possess besides their improved antifogging action in respect to common used antifoggants also spectral sensitizing properties for light-sensitive silver halide. A particular useful spectral sensitization is obtained by applying compounds of the 45. the emulsion and the desired effect, usually said com-chloride-bromide emulsions.



(II)

wherein:

Z<sub>1</sub> represents the necessary atoms to close a heterocyclic nucleus of the thiazole series (e.g. thiazole, 4-(p-tolyl)-thiazole, 4,5-diphenylthiazole, 4-m-nitrophenylthiazole, 4-p-bromophenylthiazole, 4 - methyl-5-ethoxycarbonyl-thiazole, benzthiazole, carboxylic acid substituted benzthiazole and sulphonic acid substituted benzthiazole) and those of the thiadiazole series (e.g. 4-phenylthiadiazole, 4-ethylthiadiadiazole, 4 - benzylthiadiadiazole and 4-benzylsulphonylthiadiazole), and

Z<sub>2</sub> has the same meaning as Z' described in general Formula I.

The addenda of the present invention can be added to 65. photographic emulsions using any of the well-known techniques in emulsion preparation. For example, they can be added in dissolved state to the silver halide emulsion, or they can be added to the emulsion in the form of a dispersion similar to techniques used to incorporate colour 70. couplers in the emulsion. The stabilizing agents are preferably added to the photographic emulsion after the final digestion or after-ripening, although they can advantageously be added prior to digestion.

The hydrazone compounds described above can be used 75. in combination with other stabilizing agents e.g. of the



3. A photographic material according to claim 1 comprising a silver halide emulsion layer containing a compound according to the following general formula:



wherein:

R is hydrogen or a methyl group,

Z represents the atoms necessary for completing a pyridine nucleus, a quinoline nucleus, a pyrimidine nucleus, a quinazoline nucleus, a phthalazine nucleus, a quinoxaline nucleus, a benzimidazole nucleus, a thiazole nucleus or a benzothiazole nucleus, and

Z' represents the atoms necessary to complete a pyridine nucleus or a quinoline nucleus.

4. A photographic silver halide material according to claim 1, wherein the said emulsion contains said compound in a ratio of 0.05 millimole to 50 millimole per mole of silver halide.

5

5. A photographic silver chloride or silver chloride-bromide material according to claim 2 containing said compound in a ratio of 0.05 millimole to 10 millimole per mole silver halide.

#### References Cited

##### UNITED STATES PATENTS

|           |        |                      |        |    |
|-----------|--------|----------------------|--------|----|
| 2,588,538 | 3/1952 | Kendall et al. _____ | 96—109 | XR |
| 2,295,008 | 9/1942 | Porter et al. _____  | 96—87  | XR |

##### FOREIGN PATENTS

|         |        |                |
|---------|--------|----------------|
| 447,109 | 5/1936 | Great Britain. |
| 636,403 | 4/1950 | Great Britain. |

15 NORMAN G. TORCHIN, Primary Examiner

M. F. KELLEY, Assistant Examiner

U.S. Cl. X.R.

20 96—109

UNITED STATES PATENT OFFICE  
CERTIFICATE OF CORRECTION

Patent No. 3,525,622 Dated August 25, 1970

Inventor(s) Jozef Frans Willems et al

It is certified that error appears in the above-identified patent and that said Letters Patent are hereby corrected as shown below:

Column 4, line 12 (Compound 11.) change "HH" etc. to HN --.

Column 5, (Compound 32.) change



Column 6, line 45, delete the entire incorrect line and substitute -- following general formula II in silver chloride and silver --.

Column 7, Table 2, line 60 (in the heading, column 3)

Change:  to --   
density fog  
density

SEARCHED  
INDEXED  
SERIALIZED  
FILED  
NOV 3 1970

(SEAL)

Attest:

Edward M. Fletcher, Jr.

Attesting Officer

WILLIAM E. SCHUYLER, JR.  
Commissioner of Patents